

## UNITED STATES PATENT OFFICE

1,953,398

## TREATMENT OF CELLULOSE ESTERS

Roderick K. Eskew, East Orange, N. J., assignor to  
 Du Pont Viscloid Company, Wilmington, Del.,  
 a corporation of Delaware

No Drawing. Application December 5, 1930,  
 Serial No. 500,432. Renewed January 23, 1934

8 Claims. (Cl. 260—143)

This invention relates to the treatment of cellulose esters, to effect stabilization, viscosity reduction; bleaching and clarification thereof. While not restricting the invention thereto, it is, for 5 definiteness, described with more particular reference to cellulose nitrate, and particularly with reference to cellulose nitrate having a nitrogen content below 12.5% as used in the lacquer and pyroxylin plastic industries.

10 In the production of nitrocellulose, an important step is the stabilization of the same, i. e. the treatment of the ester with water at a temperature as closely approaching the boiling point as is practicable in factory operations, in order to 15 hydrolyze such unstable esters, e. g. cellulose sulphate, as may be present in the product. Also, it is frequently desired to reduce the viscosity of nitrocellulose while in its undissolved state, either colloided or uncolloided. By reducing the 20 viscosity of the nitrocellulose, I of course mean that the nitrocellulose is so changed that a composition thereof containing a certain amount of nitrocellulose, will have a lower viscosity than a like composition containing an equal amount 25 of the cellulose nitrate untreated to lower its viscosity characteristic. A desirable way of reducing viscosity, is to treat the nitrocellulose in the presence of a direct source of oxygen, such for example as a peroxide, perborate, or the like, 30 having the characteristic that it will give up free oxygen under proper conditions.

I have devised a process whereby the viscosity of a cellulose ester e. g. cellulose nitrate, may be reduced by treatment involving the use of a direct source of oxygen; and furthermore I have devised a process wherein this treatment may be satisfactorily carried on simultaneously with, in practical effect, as an integral part of the stabilization treatment.

40 One object of the invention is to provide a process for the reduction of the viscosity of a cellulose ester, by treatment employing the use of a direct source of oxygen. A further object is to provide a combined stabilization and viscosity 45 reduction process, such process preferably further including the feature of bleaching and clarifying the cellulose ester. A further object is to provide a process for the stabilization and viscosity reduction which may be carried on at atmospheric pressure. To these ends and also to 50 improve generally on processes of the general character indicated, the invention consists in the various matters hereinafter described and claimed.

55 In accordance with the invention, as preferably

practiced, the stabilization and the viscosity reduction are carried on simultaneously, my discoveries, and the practical application of those discoveries, permitting and providing for the successful accomplishment of this end. A desirable 60 way of affecting this, is to treat cellulose nitrate with hot water containing e. g. hydrogen peroxide as a direct source of oxygen, and an alkali, e. g. sodium hydroxide as an agent for increasing the activity of the peroxide. An important feature is that although the peroxide can be used in such small amounts that its consumption in the process is not a disadvantageous feature, the viscosity reducing action is highly satisfactory. And furthermore, as previously indicated this result can be effected at temperature 70 sufficiently high to insure satisfactory stabilization.

By way of illustration merely, and not by way of limitation, the following will serve as an example of practice in accordance with the invention. Prior to treatment in accordance with the example, the nitrocellulose is nitrated in the usual way to obtain a product of approximately 11.2% nitrogen content and for reasons of economy a 80 high viscosity, say 2000 cps., and is drowned in the usual manner in a large amount of water, and the excess acid water drained off:—

The nitrocellulose was given two or three washes with water for the purpose of removing the greater portion of the retained acid. After draining there was added, in the approximate proportion of 20 parts of liquid to one part of 90 pyroxylin, an aqueous solution containing .80% hydrogen peroxide. In order to neutralize the residual traces of acid in the nitrocellulose and also the acid normally associated with hydrogen peroxide, there was added to the bath sufficient 95 dilute sodium hydroxide solution to bring the bath to neutrality. There was then added sufficient sodium hydroxide in water solution to give a concentration of .15% sodium hydroxide. The mixture was then heated at atmospheric pressure 100 to a temperature of 85° to 90° C. After one hour at this temperature the viscosity was reduced to 154 cps. Furthermore the cellulose nitrate was thoroughly bleached and its stability to the methyl violet paper test at 134.5° C. was 40 105 minutes. In addition the solubility and clarity in the camphor alcohol mixtures commonly employed with this type nitrocellulose was greatly improved.

While, in the above example, a proportion of 110

solution to nitrocellulose of 20 to 1 is mentioned it will be understood that this liquid-to-solid ratio is not essential to the chemistry of the process, since any convenient ratio may be used, 5 say, from 10 to 1 up to 30 to 1, or higher, governed largely by the type of equipment used in the handling of the mixture, the considerations being that there shall be sufficient solution to satisfactorily cover and permeate the nitrocellulose, and 10 like operating factors. 20 to 1 is a convenient ratio where the type poacher or boiling tub commonly employed in nitrocellulose purification is used.

Hydrogen peroxide is mentioned because of 15 its leaving no residue. However, other soluble comparable oxidizing agents such as perborates (e. g. sodium perborate) percarbonates (e. g. sodium percarbonate) and so forth, may be used. It will be noted that, in consideration of the other 20 features of the process, the use of oxidizing compounds which are particularly active in alkaline mediums is, generally speaking, to be preferred. Furthermore, while the use, and addition, of hydrogen peroxide as such is referred to in the 25 example, it will be plain that if for any reason it be desired, the peroxide can be generated in the solution, as by the use of sodium peroxide and an acid.

In place of the particular alkali, sodium hydroxide, mentioned in the example, there may, of course, be used various other alkalies. Thus, there may be used such other water soluble compounds as will develop a sufficient alkalinity (i. e. a pH greater than 7.0) to produce the desired 35 activity of the peroxide; e. g. sodium carbonate,  $\text{NH}_3$  etc.

Referring to the giving of a definite alkalinity to the solution as mentioned in the example, it will be understood that the alkalinity can be 40 widely varied from, and greater or less than, that mentioned in the example. A particular consideration is that the alkalinity of the solution should be sufficient to insure that the compound serving as the direct source of oxygen, e. g. hydrogen peroxide, be given an adequate activity. Also, the concentration of the direct source of oxygen may be considerably varied from the figure given in the example. It is, however, desirable to use a 45 concentration which, in consideration of the particular concentration of alkali that may be used, will bring about the desired reduction in viscosity in, at most, the time which would be required for adequate stabilization. Furthermore, the concentration of the peroxide and/or alkali may be so 50 far increased that the desired reduction in viscosity can be effected in less than the time required for stabilization merely. The practical effect of this is, that, if desired, the viscosity reduction may occupy but a portion of the stabilizing period. 55 That is, the viscosity reducing items, e. g. sodium hydroxide and hydrogen peroxide, may be added to the water, at the beginning of the stabilizing treatment or later on. Care should be taken of course that, when the introduction of the viscosity reducing items is delayed, the desired reduction shall be effected by the time stabilization 60 be completed. This procedure is more particularly applicable to, although not necessarily confined to, the treatment of pyroxylin of approximately 65 12% nitrogen content.

While it would at first appear to one skilled in the art that the use of the alkali would bring about the permanent discoloration of the cellulose ester under treatment, I have found it to be the fact that this is not the case. In fact, the cellulose

ester at the completion of the treatment will be found to be of exceptionally good color.

Of course, after the completion of the stabilizing and viscosity reducing treatment, and after the liquor has been drained off (for re-use if it contains peroxide) such alkali as remains in the ester, should be neutralized, as by the addition of a small quantity of any suitable acid, or a short acid boil, after which the ester is water-washed free from the treating solution. In certain cases 85 the acid liberated from the nitrocellulose on account of its hydrolysis will be sufficient to neutralize the alkali by the time the normal end of the treatment is reached; and, obviously, in such cases the subsequent acid treatment becomes unnecessary. At the completion of the entire treatment, the fully treated product is thoroughly water washed.

In further illustration of the process the following examples may be cited:—

## II

The nitrocellulose, and all the conditions in this example were the same as those in Example I except that at the beginning of the treatment the 100 concentration of hydrogen peroxide was .40% and the concentration of sodium hydroxide .30%, and except that treatment was prolonged for six hours. After treating for one hour the viscosity had been reduced to 81 cps. and after six hours 105 treatment it had been reduced to 60 cps. The stability by the methyl violet paper test at 134.5° C. was 40 minutes. The color of the nitrocellulose and its clarity in camphor alcohol solution were equally as good as the result obtained in the 110 case of Example I.

## III

The nitrocellulose, and all the conditions of the treatment were the same as in Example I except 115 that the concentration of hydrogen peroxide was .40% and the treatment was prolonged for six hours. At the end of one hour's treatment the viscosity had been reduced to 238 cps. and the peroxide concentration to .03% and after six 120 hours treatment it was 150 cps. and the peroxide had been entirely consumed.

## III<sup>a</sup>

The nitrocellulose and the conditions in this 125 example were the same as those in Example III except that the addition of the hydrogen peroxide to the bath was postponed until the nitrocellulose had been subjected to treatment for  $\frac{1}{2}$  hour at the temperature indicated (85° to 90° C.) with the 130 alkali. The peroxide was then added. After one hour's treatment ( $\frac{1}{2}$  hour with alkali plus  $\frac{1}{2}$  hour with peroxide and alkali) the viscosity had been reduced to 204 cps. and the peroxide concentration had fallen but to .39%. After six 135 hours total time of treatment the viscosity was 136 cps. and the peroxide had been entirely consumed.

## IV

Scrap transparent cellulose nitrate plastic (i. e. 140 a cellulosic nitrate product of about, parts by weight, colloided nitrocellulose (approximately 12% nitrogen) 100, camphor 34, ethyl alcohol 2,) cut into small pieces, was: steeped at 85° to 90° C. in a liquor containing .30% sodium hydroxide and 145 .80% hydrogen peroxide. The addition of the hydrogen peroxide was delayed until the caustic steep had been carried out for one hour. After three hours total steep (one hour with caustic plus two hours with caustic plus peroxide) the 150

viscosity of the plastic had been reduced to 476 cps. and after five and one half hours total treatment (one hour with caustic plus four and one half hours with caustic plus peroxide) the viscosity was 354 cps. The viscosity of the plastic before treatment was 1225 cps.

In the above examples, Example II illustrates, in comparison with Example I the effect of using one half the amount of peroxide and double the amount of alkali. Example III<sup>A</sup> in comparison with III illustrates the saving of peroxide which may be effected by delaying the introduction thereof in cases wherein but a short treatment, e. g. one hour, is to be given. Example IV illustrates the application of the process to the reduction of the viscosity of cellulose nitrate in the colloided state.

In the carrying out of the examples occasional stirring was used in order to insure uniformity throughout the mass, and, generally speaking, a procedure of this general type is desirable. I have found it particularly satisfactory to provide a circulation of the liquid from top to bottom of the container, by slowly drawing off the liquid at the bottom of the container and returning it to the top.

As previously suggested, it is desirable to work at a temperature which will insure the completion of stabilization in a relatively short time. The higher the temperature, the shorter will be the time required for stabilization; but I have found it the better practice to use a temperature somewhat below 100° C. to insure that the activity of the viscosity reducing factors will not become so great as to make accurate control unduly difficult. On the other hand, a temperature not substantially lower than 60° C. is desirable if the treatment is not to require an undue length of time.

I may note that the viscosities of the cellulose nitrate of approximately 11% nitrogen content, used in the examples, were measured as follows: 20 grams of the dry nitrocellulose were dissolved in 313 grams of a solvent consisting of 30% camphor by weight in ethyl alcohol; and the viscosity in centipoises equals 34 times the time in seconds required for a  $\frac{1}{8}$ " diameter aluminum sphere to fall through 10 inches of the solution in a  $1\frac{1}{8}$ " inside diameter tube at 25° C.

While the invention has been discussed with more particular reference to cellulose nitrate, it will be seen that it, in certain aspects, may be applicable to other cellulose esters, e. g. cellulose acetate. Furthermore, while the treatment of cellulose nitrate of a nitrogen content of about 11% has been particularly exemplified, it will be evident that the invention is entirely applicable to cellulose nitrate of a higher or a lower nitrogen content. However, when a higher nitrogen content is in question, an increase in the severity of the conditions, such as higher concentration of alkali and peroxide, a longer time of treatment, etc., is recommended.

I claim:

1. The method of treating a cellulose ester which comprises heating the ester in an undissolved state in an aqueous medium having a distinct alkalinity, in the presence of hydrogen peroxide. 80

2. The process of reducing the viscosity of cellulose nitrate which comprises heating the nitrate in an undissolved state in water containing hydrogen peroxide, and sodium hydroxide in quantity sufficient to give the solution a distinct alkalinity. 85

3. The process of reducing the viscosity of cellulose nitrate which comprises heating the nitrate in an undissolved state to a temperature above 60° C. in water containing hydrogen peroxide, and sodium hydroxide in quantity sufficient to give the solution a distinct alkalinity. 90

4. The process of reducing the viscosity of cellulose nitrate which comprises heating the nitrate in an undissolved state to a temperature substantially between 80° C. and 95° C. in water containing hydrogen peroxide, and sodium hydroxide in quantity sufficient to give the solution a distinct alkalinity. 95

5. The process of treating unstabilized cellulose nitrate to stabilize the same and reduce the viscosity thereof which process comprises immersing unstabilized cellulose nitrate in the undissolved state in water containing hydrogen peroxide and an alkali in sufficient quantity to give the solution a distinct alkalinity, heating at substantially 80° C. to 95° C. to effect hydrolysis of unstable esters and viscosity reduction, and removing hydrolyzed esters and residual re-agents. 105

6. The process of treating unstabilized cellulose nitrate to stabilize the same and reduce the viscosity thereof which process comprises immersing unstabilized cellulose nitrate in the undissolved state in water containing hydrogen peroxide and an alkali in sufficient quantity to give the solution a distinct alkalinity, heating at substantially 80° C. to 95° C. to effect hydrolysis of unstable esters and viscosity reduction, draining and washing. 115

7. The process of treating unstabilized cellulose nitrate to stabilize the same and reduce the viscosity thereof which process comprises immersing unstabilized cellulose nitrate in the undissolved state in water containing hydrogen peroxide and an alkali in sufficient quantity to give the solution a distinct alkalinity, heating at substantially 80° C. to 95° C. to effect hydrolysis of unstable esters and viscosity reductions, draining, adding acid to neutralize any retained alkali, and washing. 125

8. The process of reducing the viscosity of cellulose nitrate which comprises heating the nitrate in an undissolved state in water containing hydrogen peroxide, and an alkali in quantity sufficient to give the solution a distinct alkalinity. 135

RODERICK K. ESKEW.